

Patented Aug. 13, 1940

Examiner  
and a small amount of stearone 64  
or chlorinated stearone 2,211,687  
 $C_{35}H_{70}$

## UNITED STATES PATENT OFFICE

2,211,687

## LUBRICATING COMPOSITION

Benjamin T. Brooks, New York, N. Y., assignor,  
by mesne assignments, to American Cyanamid  
Company, New York, N. Y., a corporation of  
Maine

X 252-54

No Drawing. Application March 18, 1937,  
Serial No. 131,628

2 Claims. (Cl. 87-9)

This invention relates to lubricating compositions and particularly to the so-called extreme pressure lubricants.

The standard lubricants for heavy duty service, that is, in internal combustion engines, are mostly hydrocarbon oils. These mineral oils when properly refined are very stable under heat but they are deficient in oiliness and in the strength of the oil film which is formed between metal surfaces in bearings or at other points where lubrication takes place. Both factors of film strength and oiliness are of great importance in the lubrication of heavy duty bearings such as are encountered in modern internal combustion engines or in gear transmissions with high tooth pressures, for example hypoid gears. Insufficient film strength will result in metal to metal contact even when an adequate quantity of lubricant is supplied to the bearing and insufficient oiliness will prevent retention of an oil film in the bearing when for any reason a lubricant supply becomes insufficient. Both deficient oiliness and deficient film strength permit metal to metal contact which results in higher wear and also in the rapid development of heat. Modern high speed internal combustion engines operate at so close to the limit of bearing pressures and rubbing speeds that it has been necessary to change the material used in the bearing, for example, to substitute certain bearing metals such as alloys containing silver, cadmium and the like, for the standard babbitt metals.

Film strength and oiliness are probably due to molecular forces in the oil film, the molecules of which have the property of wetting or adhering to the metal surface. An oil film is retained tenaciously even when the lubricant supply is interrupted for considerable periods of time.

In the past, the problem was first attacked by the incorporation of small amounts of fatty acids into the oil. These compounds did in fact increase the oiliness to some extent but they did not produce films of high strength and corrosion and other difficulties rendered their use undesirable. Certain esters such as tricresyl and triphenylphosphate and chlorinated esters of fatty acids with mono or dihydric alcohols have been proposed and have achieved some commercial success, notably in the case of tricresylphosphate and chlorinated stearic acid esters. The presence of the acid radical even though combined in ester form was therefore considered to be a desirable component group of such compounds.

According to the present invention, I have

found that ketones obtainable by combining long chain fatty acids such as oleic, stearic, palmitic and the like, or by combining the mixtures of acids obtained from cottonseed oil, lard oil, stearine, fish oil and tallow, and the like, when blended with lubricating oils or greases increase the film strength notably and greatly increase the oiliness of the products. These ketones are very stable under heat and are not corrosive to metals.

The higher molecular unsubstituted ketones have the advantage over other substances used to increase film strength and oiliness in that they do not contain any halogen and therefore cannot decompose to yield hydrochloric acid.

While the halogen free ketones are very effective and possess the advantage that they contain no constituents which form hydrochloric acid, higher film strengths may be obtained when the products are chlorinated. It is thus possible in the chlorinated products of the present invention to obtain the advantages and increased film strength which halogen containing compounds offer, without excessive danger from corrosion due to possible formation of hydrochloric acid in use. When unsaturated ketones, such as oleones, are chlorinated the chlorine adds to the double bonds and di and tetra chloroleones are produced. Such chlorinated ketones are not as stable as the monochlorinated products. They can be transformed into highly stable compounds by heat or preferably by treatment with sufficient caustic soda to remove one chlorine atom as hydrochloric acid, HCl, from the dichlor product or two chlorine atoms from the tetrachlor product. The partly dechlorinated products in which the chlorine is adjacent to an unsaturated or olefin group are highly stable and the advantage of the chlorinated product may be obtained without corrosion dangers. Mixtures containing ketones of the order of 1% give sufficient increase in film strength and oiliness. Larger amounts can, of course, be used, but the factor of diminishing returns soon enters and the advantage obtained by adding very large quantities of the ketones do not offset the increase in cost for, of course, the ketones are much more expensive than the lubricating oil base itself.

The ketone of the present invention are usable with lubricating oils and greases of the most varying characteristics. The improvement in film strength and particularly in oiliness will, however, in general, differ with different mineral oils. Thus, for example, with a mineral oil stock which has been refined by solvents to such an extent

that it has lost most of its oiliness, the addition of the ketones of the present invention will make a much bigger difference than in the case of a mineral oil where the oiliness has not been so 5 completely removed. It should also be understood that the varying purposes for which the lubricating composition is to be employed determine to a large extent the particular ketone which is to be used. Thus, for example, in the gear lubricants for hypoid gears, the film strength is of the 10 greatest importance and since the temperature of operation is relatively low, danger of decomposition of halogen containing compounds with the setting free of halogen acids is not a serious factor. Chlorinated ketones may be used which, in 15 general, show a higher film strength. On the other hand, in the case of lubricating oil for internal combustion engines, where the operating temperatures are high and danger of decomposition greater, it is sometimes preferable to use 20 unhalogenated ketones of the present invention which possess high degrees of oiliness with lower film strengths.

Other uses may emphasize one or other of the 25 characteristics and in each case the ketone having the best general characteristics for the particular use should be chosen. It is an advantage of the present invention that a wide choice of ketones halogenated and unhalogenated is available. While the halogenated ketones possess substantially similar properties, whether the halogen is fluorine, chlorine or bromine, the bromine compounds are much more expensive and for the most purposes therefore the chlorine compounds 30 are preferable because of the large saving in cost.

The invention will be described in greater detail in conjunction with the following specific examples which are typical illustrations of uses of the compounds of the present invention.

#### 40. Example 1

.1% of stearone was added to a standard mineral lubricating oil for internal combustion engines and tested on the lubricant tester developed by the Bureau of Standards with a high speed test specimen of 2500 R. P. M. and low speed specimen of 938 R. P. M., giving a speed ratio of 8:3. The rate of loading increased about 45 12 lbs. per second and the initial oil temperature was 75° F. Under these conditions, the mixture showed a load carrying capacity of 185 lbs. as compared to 148 lbs. for the oil without ketone. A marked increase in oiliness can be noted.

#### 55. Example 2

Chlorinated stearone containing one atom of chlorine per mole was mixed with the same mineral oil as described in Example 1 and tested. A 1% solution gave a film strength of 185 under

more drastic conditions, involving a speed ratio of 5:1 instead of 8:3. The chlorinated compound, while giving very satisfactory film strengths, requires somewhat larger amounts. These larger amounts, however, confer a higher degree of oiliness so that a 1% chlorinated stearone mixture in some respects is distinctly superior to a 1% of stearone solution. Chlorinated stearone is also more soluble in mineral oils than stearone.

#### 10. Example 3

Chlorinated oleone and stearone were tested in a 1% solution in a naphthenic base oil on a different type of machine, namely, an Amsler machine which has a maximum reading of 300 lbs. Both 15 mixtures showed a maximum film strength of 300 lbs. at a torque of 75 lbs. for the chlorinated oleone and 58 lbs. for the chlorinated stearone. The Amsler machine not only measures film strength but gives a rough comparison of oiliness. Tricresylphosphate which is a standard addition to lubricants to endow them with extreme pressure characteristics when used in a 1% solution in the same naphthenic base oil as the chlorinated stearone and oleone above referred to, gave a film strength of 160 lbs. with a torque of 68. When the amount of tricresylphosphate was increased to 2% the film strength rose to 200 lbs. with an increase of torque to 80. It will be apparent that at a much higher loading 30 the chlorinated stearone gave a lower torque and hence was more oily than the 1% tricresylphosphate solution and the chlorinated oleone at a 50% higher load gave somewhat lower torque than the 2% tricresylphosphate solution. 35

It is an advantage of the present invention that the addition of the chlorinated ketones does not raise the pour point of the lubricant and most of them lower the pour point, which is, of course, of great advantage as material savings in refining 40 cost can be enjoyed if the added compounds exert sufficient lowering of pour point to make the less refined oil meet the normal requirements. Similarly the pour point depressing effect of the compounds of the present invention may be used 45 with oils which already have a very low pour point due to very thorough removing of wax, thus producing products which have pour points lower than ordinarily specified which special oils can then be used for extreme cold weather 50 operation.

I claim:

1. A lubricating composition comprising a mineral lubricant and a small amount of stearone.
2. A lubricating composition comprising a 55 mineral lubricant and a small amount of chlorinated stearone.

BENJAMIN T. BROOKS.